# EUROPEAN PATENT APPLICATION

(11) **EP 1 876 496 A2**
(43) Date of publication of application: **09.01.2008**
(21) Application number: 07111993.7
(22) Date of filing: 06.07.2007
(51) Int. Cl.: G03G 5/06

(54) **Imaging members and method for sensitizing a charge generation layer of an imaging member**

(30) Priority: 06.07.2006 US 481762
(71) Applicant: Xerox Corporation, Rochester, New York 14644 (US)
(72) Inventor: Wu, Jin, Webster, NY 14580 (US); Wilbert, John J., Macedon, NY 14502 (US); Ferrarese, Linda L., Rochester, NY 14612 (US); Lin, Liang-Bih, Rochester, NY 14618 (US)
(74) Representative: Jones, Helen M.M.

(57) **Abstract**

An imaging member including a substrate; an optional undercoat layer; a charge generating layer comprising photoconductive pigment and a pigment sensitizing dopant having an electron acceptor molecule; and a charge transport layer.

## Description

The present disclosure is generally related to imaging members, also referred to as photoreceptors, photosensitive members, and the like, and in embodiments to methods of treating the charge generation layer of electrophotographic imaging members. The imaging members may be used in copy, printer, fax, scan, multifunction machines, and the like. In embodiments, the methods reduce scratching, abrasion, corrosion, fatigue, and cracking, and facilitate cleaning and durability of devices, for example active matrix imaging devices, such as active matrix belts.

In the art of electrophotography, a photoreceptor, imaging member, or the like, comprising a photoconductive insulating layer on a conductive layer is imaged by first uniformly electrostatically charging the surface of the photoconductive insulating layer. The photoreceptor is then exposed to a pattern of activating electromagnetic radiation such as light, which selectively dissipates the charge in the illuminated areas of the photoconductive insulating layer while leaving behind an electrostatic latent image in the non-illuminated areas. This electrostatic latent image may then be developed to form a visible image by depositing finely divided electroscopic toner particles on the surface of the photoconductive insulating layer. The resulting visible toner image can be transferred to a suitable receiving member such as paper. This imaging process may be repeated many times with reusable photoconductive insulating layers.

Electrophotographic imaging members or photoreceptors are usually multilayered photoreceptors that comprise a substrate support, an electrically conductive layer, an optional hole blocking layer, an optional adhesive layer, a charge generating layer, and a charge transport layer in either a flexible belt form or a rigid drum configuration. Multilayered flexible photoreceptor members may include an anti-curl layer on the backside of the substrate support, opposite to the side of the electrically active layers, to render the desired photoreceptor flatness.

Examples of photosensitive members having at least two electrically operative layers including a charge generating layer and diamine containing transport layer are disclosed in U. S. Patent Numbers 4,265,990; 4,233,384; 4,306,008; 4,299,897; and 4,439,507.

Photoreceptors can also be single layer devices. For example, single layer organic photoreceptors typically comprise a photogenerating pigment, a thermoplastic binder, and hole and electron transport materials.

As more advanced, higher speed electrophotographic copiers, duplicators and printers were developed, the performance requirements for the xerographic components increased. Moreover, complex, highly sophisticated, duplicating and printing systems employing flexible photoreceptor belts, operating at very high speeds, have also placed stringent mechanical requirements and narrow operating limits as well on photoreceptors.

The charge generating layer is capable of photogenerating holes and injecting the photogenerated holes into the charge transport layer. The charge generating layer used in multilayered photoreceptors include, for example, inorganic photoconductive particles or organic photoconductive particles dispersed in a film forming polymeric binder. Inorganic or organic photoconductive material may be formed as a continuous, homogenous charge generation section. Many suitable photogenerating materials known in the art may be used, if desired.

Electrophotographic imaging members or photoreceptors having varying and unique properties are needed to satisfy the vast demands of the xerographic industry. The use of organic photogenerating pigments such as perylenes, bisazos, perinones, and polycyclic quinines in electrophotographic applications is well known. Generally, layered imaging members with the aforementioned pigments exhibit acceptable photosensitivity.

However, faster pigments are desired for future photoreceptor device designs as process speeds increase.

Common print quality issues are strongly dependent on the quality of the charge generation layer. For example, charge deficient spots and bias charge roll leakage breakdown are problems that commonly occur. Another problem is imaging ghosting which is thought to result from the accumulation of charge somewhere in the photoreceptor. Consequently, when a sequential image is printed, the accumulated charge results in image density charges in the current printed image that reveals the previously printed image.

U. S. Patent 6,350,550, describes in the Abstract thereof a charge generation section of an electrophotographic imaging member having hydroxygallium phthalocyanine photoconductive pigment and benzimidazole perylene photoconductive pigment in a solvent solution comprising a film forming polymer or copolymer dissolved in a solvent.

U. S. Patent 6,063,553, describes in the Abstract thereof an electrophotographic imaging member including a supporting substrate; an undercoat layer; a charge generating layer comprising photoconductive pigment particles, film forming binder and a charge transport layer formed from a coating solution, the coating solution comprising charge transporting molecules, the charge transporting molecules comprising a major amount of a first charge transport molecule comprising an alkyl derivative of an arylamine and a minor amount of second transport molecule comprising an alkyloxy derivative of an arylamine, the charge generating layer being located between the substrate and the charge transport layer. A process for fabricating this imagine member is also disclosed.

U. S. Patent 5,350,654, describes in the Abstract thereof a layered photoreceptor composed of a substrate, an extrinsic pigment layer that has been sensitized disposed over the substrate, and a charge transport polymer in contact with the pigment layer. A method for producing a photoreceptor comprises depositing a layer of sensitizing electron donor material in a polymer binder on a substrate. An extrinsic pigment layer is deposited on the layer of sensitizing electron donor material. A charge transport layer is deposited on the pigment layer.

The present invention relates to an imaging member comprising a substrate; an optional undercoat layer; a charge generating layer comprising photoconductive pigment and a pigment sensitizing dopant having an electron acceptor molecule; and at least one charge transport layer.

In a further aspect of the invention there is provided a process for fabricating an imaging member comprising providing a substrate; forming an optional undercoat layer on the substrate; forming a sensitized charge generation layer comprising photoconductive pigment and a pigment sensitizing dopant having an electron acceptor molecule; and forming at least one charge transport layer. In embodiments, for example, the charge generation layer comprises a photoconductive pigment, a polymeric resin and a pigment sensitizing dopant having an electron acceptor molecule.

Embodiments disclosed herein further include a process for fabricating an imaging member exhibiting low imaging ghosting.

In a further aspect the present invention relates to an image forming apparatus for forming images on a recording medium comprising a) a photoreceptor member having a charge retentive surface to receive an electrostatic latent image thereon, wherein said photoreceptor member comprises a metal or metallized substrate, a charge generating layer, and at least one charge transport layer; wherein the charge generating layer comprises a photoconductive pigment and a pigment sensitizing dopant having an electron acceptor molecule; b) a development component to apply a developer material to said charge-retentive surface to develop said electrostatic latent image to form a developed image on said charge-retentive surface; c) a transfer component for transferring said developed image from said charge-retentive surface to another member or a copy substrate; and d) a fusing member to fuse said developed image to said copy substrate.

Any suitable multilayer photoreceptor may be employed. The various layers may be applied in any suitable order to produce either positive or negative charging photoreceptors. The charge generating layer may be applied prior to the charge transport layer, or the charge transport layer may be applied prior to the charge generating layer. In embodiments, the first pass charge transport layer is formed upon a charge generating layer and the second pass charge transport layer is formed upon the first pass charge transport layer.

The supporting substrate can be selected to include a conductive metal substrate or a metallized substrate. While a metal substrate is substantially or completely metal, the substrate of a metallized substrate is made of a different material that has at least one layer of metal applied to at least one surface of the substrate. The material of the substrate of the metallized substrate can be any material for which a metal layer is capable of being applied. The substrate can be a synthetic material, such as a polymer. In embodiments, a conductive substrate is, for example, at least one member selected from the group consisting of aluminum, aluminized or titanized polyethylene terephthalate belt (Mylar®).

Any metal or metal alloy can be selected for the metal or metallized substrate. Typical metals employed for this purpose include aluminum, zirconium, niobium, tantalum, vanadium, hafnium, titanium, nickel, stainless steel, chromium, tungsten, molybdenum, mixtures and combinations thereof, and the like. Useful metal alloys may contain two or more metals such as zirconium, niobium, tantalum, vanadium, hafnium, titanium, nickel, stainless steel, chromium, tungsten, molybdenum, mixtures and combinations thereof, and the like. Aluminum, such as mirror-finish aluminum, is selected in embodiments for both the metal substrate and the metal in the metallized substrate. All types of substrates may be used, including honed substrates, anodized substrates, bohmite-coated substrates and mirror substrates.

Examples of substrate layers include opaque or substantially transparent materials, and may comprise any suitable material having the requisite mechanical properties. For example, the substrate can comprise a layer of insulating material including inorganic or organic polymeric materials, such as Mylar®, Mylar® containing titanium, a layer of an organic or inorganic material having a semiconductive surface layer, such as indium tin oxide or aluminum arrange thereon, or a conductive material such as aluminum, chromium, nickel, brass or the like. The substrate may be flexible, seamless, or rigid, and may have a number of different configurations, for example, a plate, a cylindrical drum, a scroll, and endless flexible belt, or other configuration. It may be desirable to provide an anticurl layer to the back of the substrate.

Optionally, a hole blocking layer is applied, to the substrate. Generally, electron blocking layers for positively charged photoreceptors allow the photogenerated holes in the charge generating layer at the top of the photoreceptor to migrate toward the charge (hole) transport layer below and reach the bottom conductive layer during the electrophotographic imaging process. Thus, an electron blocking layer is normally not expected to block holes in positively charged photoreceptors such as photoreceptors coated with a charge generating layer over a charge (hole) transport layer. For negatively charged photoreceptors, any suitable hole blocking layer capable of forming an electronic barrier to holes between the adjacent photoconductive layer and the underlying substrate layer may be utilized. Typical hole blocking layers utilized for the negatively charged photoreceptors may include, for example, polyamides such as Luckamide® (a nylon-6 type material derived from methoxymethyl-substituted polyamide), hydroxyl alkyl methacrylates, nylons, gelatin, hydroxyl alkyl cellulose, organopolyphosphazenes, organosilanes, organotitanates, organozirconates, silicon oxides, zirconium oxides, zinc oxides, titanium oxides, and the like. In embodiments, the hole blocking layer comprises nitrogen containing siloxanes.

The blocking layer, as with all layers herein, may be applied by any suitable technique such as, but not limited to, spraying dip coating, draw bar coating, gravure coating, silk screening, air knife coating, reverse roll coating, vacuum deposition, chemical treatment, and the like.

An adhesive layer may optionally be applied such as to the hole blocking layer. The adhesive layer may comprise any suitable material, for example, any suitable film forming polymer. Typical adhesive layer materials include, but are not limited to, copolyester resins, polyarylates, polyurethanes, blends of resins, and the like. Any suitable solvent may be selected to form an adhesive layer coating solution, including, but not limited to, tetrahydrofuran, toluene, hexane, cyclohexane, cyclohexanone, methylene chloride, 1,1,2-trichloroethane, monochlorobenzene, and mixtures thereof, and the like.

The photogenerating or charge-generating component converts light input into electron hole pairs. Examples of compounds suitable for use as the charge-generating component include vanadyl phthalocyanine, metal phthalocyanines (such as titanyl phthalocyanine, chlorogallium phthalocyanine, hydroxygallium phthalocyanine, and alkoxygallium phthalocyanine), metal-free phthalocyanines, benzimidazole perylene, amorphous selenium, trigonal selenium, selenium alloys (such as selenium-tellurium, selenium-tellurium arsenic, selenium arsenide), chlorogallium phthalocyanine, and mixtures and combinations thereof. In embodiments, a photogenerating layer includes metal phthalocyanines and/or metal free phthalocyanines, at least one phthalocyanine selected from the group consisting of titanyl phthalocyanines, perylenes, or hydroxygallium phthalocyanines, Type V hydroxygallium phthalocyanine, Type A, B or C chlorogallium phthalocyanine, Type IV titanyl phthalocyanine, or Type V titanyl.

Illustrated in U.S. Patent 5,521,306, is a process for the preparation of Type V hydroxygallium phthalocyanine comprising the in situ formation of an alkoxy-bridged gallium phthalocyanine dimer, hydrolyzing the dimer to hydroxygallium phthalocyanine and subsequently converting the hydroxygallium phthalocyanine product to Type V hydroxygallium phthalocyanine.

Illustrated in U.S. Patent 5,482,811, is a process for the preparation of hydroxygallium phthalocyanine photogenerating pigments which comprises hydrolyzing a gallium phthalocyanine precursor pigment by dissolving the hydroxygallium phthalocyanine in a strong acid and then reprecipitating the resulting dissolved pigment in basic aqueous media; removing any ionic species formed by washing with water, concentrating the resulting aqueous slurry comprised of water and hydroxygallium phthalocyanine to a wet cake; removing water from said slurry by azeotropic distillation with an organic solvent, and subjecting said resulting pigment slurry to mixing with the addition of a second solvent to cause the formation of said hydroxygallium phthalocyanine polymorphs.

U.S. Patent 5,473,064, illustrated a process for the preparation of photogenerating pigments of hydroxygallium phthalocyanine Type V essentially free of chlorine, whereby a pigment precursor Type I chlorogallium phthalocyanine is prepared by reaction of gallium chloride in a solvent, such as N-methylpyrrolidone, present in an amount of from about 10 parts to about 100 parts, and preferably about 19 parts with 1,3-diiminoisoindolene (DI³) in an amount of from about 1 part to about 10 parts, and preferably about 4 parts of DI³, for each part of gallium chloride that is reacted; hydrolyzing said pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts and preferably about 15 volume parts for each weight part of pigment hydroxygallium phthalocyanine that is used by, for example, ball milling the Type I hydroxygallium phthalocyanine pigment in the presence of spherical glass beads, approximately 1 mm to 5 mm in diameter, at room temperature, about 25°C, for a period of from about 12 hours to about 1 week, and preferably about 24 hours.

A number of titanyl phthalocyanines, or oxytitanium phthalocyanines, are suitable photogenerating pigments known to absorb near infrared light around 800 nanometers and have exhibited improved sensitivity compared to other pigments such as, hydroxygallium phthalocyanine. Titanyl phthalocyanine is known to have five main crystal forms known as Types I, II, III, X, and IV. The various polymorphs of titanyl phthalocyanine have been demonstrated as suitable pigments in the charge or photogenerating layer of a photoimaging member or device. Various methods for preparing a titanyl phthalocyanine having a particular crystal phase have been demonstrated.

The titanyl phthalocyanines selected for the photogenerating layer exhibit a crystal phase that is distinguishable from other known titanyl phthalocyanine polymorphs, and are designated as Type V polymorphs. The processes generally comprises converting a Type I titanyl phthalocyanine to a Type V titanyl phthalocyanine pigment. The processes include converting a Type I titanyl phthalocyanine to an intermediate titanyl phthalocyanine, which is designated as a Type Y titanyl phthalocyanine, and then subsequently converting the Type Y titanyl phthalocyanine to a Type V titanyl phthalocyanine.

In one embodiment, the process comprises: (a) dissolving a Type I titanyl phthalocyanine in a suitable solvent; (b) adding the solvent solution comprising the dissolved Type I titanyl phthalocyanine to a quenching solvent system to precipitate an intermediate titanyl phthalocyanine (designated as a Type Y titanyl phthalocyanine); and (c) treating the resultant Type Y phthalocyanine with a halo, such as, for example, monochlorobenzene to obtain a resultant high sensitivity titanyl phthalocyanine, which is designated herein as a Type V titanyl phthalocyanine. In another embodiment, prior to treating the Type Y phthalocyanine with a halo, such as monochlorobenzene, the Type Y titanyl phthalocyanine may be washed with various solvents including, for example, water, and/or methanol. The quenching solvents system to which the solution comprising the dissolved Type I titanyl phthalocyanine is added comprises an alkyl alcohol and an alkylene halide.

The process further provides a titanyl phthalocyanine having a crystal phase distinguishable from other known titanyl phthalocyanines. The titanyl phthalocyanine prepared by a process according to the present disclosure, which is designated as a Type V titanyl phthalocyanine, is distinguishable from, for example, Type IV titanyl phthalocyanines, in that a Type V titanyl phthalocyanine exhibits an x-ray powder diffraction spectrum having four characteristic peaks at 9.0°, 9.6°, 24.0°, and 27.2°, while Type IV titanyl phthalocyanines typically exhibit only three characteristic peaks at 9.6°, 24.0°, and 27.2°.

Any Type I titanyl phthalocyanine may be selected as the starting material in the present process. Type I titanyl phthalocyanines suitable for use in the present process may be obtained by any suitable method.

A Type I titanyl phthalocyanine may be prepared, in one embodiment by the reaction of DI³ (1,3-diiminoisoindolene) and tetrabutoxide in the presence of 1-chloronaphthalene solvent, whereby there is obtained a crude Type I titanyl phthalocyanine, which is subsequently purified, up to about a 99.5 percent purity, by washing with, for example, dimethylformamide.

In another embodiment, a Type I titanyl phthalocyanine can be prepared by i) the addition of 1 part titanium tetrabutoxide to a stirred solution of from about 1 to about 10 parts and, in embodiments, about 4 parts of 1,3-diiminoisoindolene; ii) relatively slow application of heat using an appropriate sized heating mantle at a rate of about 1 to about 10 degrees per minute and, in embodiments, about 5 degrees per minute until refluxing occurs at a temperature of about 130 to about 180°C; iii) removal and collection of the resulting distillate, which was shown by NMR spectroscopy to be butyl alcohol, in a dropwise fashion, using an appropriate apparatus such as a Claisen Head condenser, until the temperature of the reactants reaches from 190 to about 230°C degrees and, in embodiments, about 200°C; iv) continued stirring at the reflux temperature for a period of about 1/2 hour to about 8 hours and, in embodiments, about 2 hours; v) cooling of the reactants to a temperature of about 130 to about 180°C, and, in embodiments about 160°C, by removal of the heat source; vi) filtration of the flask contents through, for example, an M-porosity (10 to 15 µm) sintered glass funnel which was preheated using a solvent which is capable of raising the temperature of the funnel to about 150°C, for example, boiling N,N-dimethylformamide in an amount sufficient to completely cover the bottom of the filter funnel so as to prevent blockage of said funnel; vii) washing the resulting purple solid by slurrying the solid in portions of boiling DMF either in the funnel or in a separate vessel in a ratio of about 1 to about 10, and preferably about 3 times the volume of the solid being washed, until the hot filtrate became light blue in color; viii) cooling and further washing the solid of impurities by slurrying the solid in portions of N,N-dimethylformamide at room temperature, about 25 degrees, approximately equivalent to about three times blue in color; ix) washing the solid of impurities by slurrying said solid in portions of an organic solvent, such as methanol, acetone, water and the like, and in this embodiment methanol, at room temperature (about 25°C) approximately equivalent to about three times the volume of the solid being washed, until the filtrate became light blue in color; x) oven drying the purple solid in the presence of a vacuum or in air at a temperature of from about 25 to about 200°C, and, in embodiments at about 70°C, for a period of from about 2 to about 48 hours and, in embodiments for about 24 hours, thereby resulting in the isolation of a shiny purple solid which was identified as being Type I titanyl phthalocyanine by its X-ray powder diffraction trace.

In another embodiment, a Type I titanyl phthalocyanine may be prepared by: (i1) reacting a DI³ with a titanium tetra alkoxide such as, for example, titanium tetrabutoxide at a temperature of about 195°C for about two hours; (ii) filtering the contents of the reaction to obtain a resulting solid; (iii) washing the solid with dimethylformamide (DMF); (iv) washing with four percent ammonium hydroxide; (v) washing with deionized water; (vi) washing with methanol; (vii) reslurrying the washes and filtering; and (viii) drying at about 70°C under vacuum to obtain a Type I titanyl phthalocyanine.

Type I titanyl phthalocyanine is dissolved in a suitable solvent. In embodiments, a Type I titanyl phthalocyanine is dissolved in a solvent comprising a trihaloacetic acid and an alkylene halide. The alkylene halide comprises, in embodiments, from about one to about six carbon atoms. Generally, the trihaloacetic acid is not limited in any manner. An example of a suitable trihaloacetic acid includes, but is not limited to, trifluoroacetic acid. In one embodiment, the solvent for dissolving a Type I titanyl phthalocyanine comprises trifluoroacetic acid and methylene chloride. In embodiments, the trihaloacetic acid is present in an amount of from about one to about 100 volume parts of the solvent and the alkylene halide is present in an amount of from about one to about 100 volume parts of the solvent. In one embodiment, the solvent comprises methylene chloride and trifluoroacetic acid in a volume-to-volume ratio of about 4 to 1. The Type I titanyl phthalocyanine is dissolved in the solvent by stirring for an effective period of time such as, for example, for about 30 seconds to about 24 hours, at room temperature. In one embodiment, the Type I titanyl phthalocyanine is dissolved by stirring in the solvent for about one hour at room temperature. The Type I titanyl phthalocyanine may be dissolved in the solvent in either air or in an inert atmosphere (e.g., argon or nitrogen).

In embodiments the Type I titanyl phthalocyanine is converted to an intermediate titanyl phthalocyanine form prior to conversion to the high sensitivity titanyl phthalocyanine pigment. "Intermediate" indicates that the Type Y titanyl phthalocyanine is a separate form prepared in the process prior to obtaining the final desired Type V titanyl phthalocyanine product. To obtain the intermediate form, which is designated as a Type Y titanyl phthalocyanine, the dissolved Type I titanyl phthalocyanine is added to a quenching system comprising an alkyl alcohol and alkylene chloride. Adding the dissolved Type I titanyl phthalocyanine to the quenching system causes the Type Y titanyl phthalocyanine to precipitate. Materials suitable as the alkyl alcohol component of the quenching system include, but are not limited to, methanol, ethanol, and the like. In embodiments, the alkylene chloride component of the quenching system comprises from about one to about six carbon atoms. In one embodiment, the quenching system comprises methanol and methylene chloride. The quenching system comprises an alkyl alcohol to alkylene chloride ratio of from about 1/4 to about 4/1 (v/v). In other embodiments, the ratio of alkyl alcohol to alkylene chloride is from about 1/1 to about 3/1 (v/v). In one embodiment, the quenching system comprises methanol and methylene chloride in a ratio of about 1/1 (v/v). In another embodiment, the quenching system comprises methanol and methylene chloride in a ratio of about 3/1 (v/v). In embodiments, the dissolved Type I titanyl phthalocyanine is added to the quenching system at a rate of from about 1 to about 100 ml/min, and the quenching system is maintained at a temperature of from about 0 to about -25°C during quenching. In a further embodiment, the quenching system is maintained at a temperature of from about 0 to about -25°C for a period of from about 0.1 hour to about 8 hours after addition of the dissolved Type I titanyl phthalocyanine solution.

Following precipitation of the Type Y titanyl phthalocyanine, the precipitates may be washed with any suitable solution, including, for example, methanol, cold deionized water, hot deionized water, and the like. Generally, washing the precipitate will also be accompanied by filtration. A wet cake containing Type Y titanyl phthalocyanine and water is obtained with water content varying from about 30 to about 70 weight percent of the wet cake.

The Type V titanyl phthalocyanine is obtained by treating the obtained intermediate Type Y titanyl phthalocyanine with a halo, such as, for example, monochlorobenzene. The Type Y titanyl phthalocyanine wet cake may be redispersed in monochlorobenzene, filtered and oven-dried at a temperature of from about 60 to about 85°C to provide the resultant Type V titanyl phthalocyanine. The monochlorobenzene treatment may occur over a period of about one to about 24 hours. In one embodiment, for a period of about five hours.

A titanyl phthalocyanine obtained, which is designated as a Type V titanyl phthalocyanine, exhibits an x-ray powder diffraction spectrum distinguishable from other known titanyl phthalocyanine polymorphs. A Type V titanyl phthalocyanine obtained exhibits an x-ray diffraction spectrum having four characteristics peaks at 9.0°, 9.6°, 24.0°, and 27.2°. A titanyl phthalocyanine prepared by in accordance with the present disclosure may have a particle size of from about 10 nm to about 500 nm. Particle size may be controlled or affected by the quenching rate when adding the dissolved Type I titanyl phthalocyanine to the quenching system and the composition of the quenching system.

The charge generating layer may comprise single or multiple layers comprising inorganic or organic compositions and the like. Suitable polymeric film-forming binder materials for the charge generating layer and/or charge generating pigment include, but are not limited to, thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, amino resins, phenylene oxide resins, terephthalic acid resins, phenoxy resins, epoxy resins, phenolic resins, polystyrene and acrylonitrile copolymers, polyvinyl chloride, vinylchloride and vinyl acetate copolymers, acrylate copolymers, alkyd resins, cellulosic film formers, poly(amideimide), styrene-butadiene copolymers, vinylidinechloride-vinylchloride copolymers, vinylacetate-vinylidenechloride copolymers, carboxyl-modified vinyl acetate-vinylchloride copolymers, styrene-alkyd resins, polyvinylcarbazole, and mixtures thereof.

The charge-generating component may also contain a photogenerating composition or pigment. The photogenerating composition or pigment may be present in the resinous binder composition in various amounts, ranging from about 5% to about 90% by volume (the photogenerating pigment is dispersed in about 10% to about 95% by volume of the resinous binder); or from about 20% to about 75% by volume (the photogenerating pigment is dispersed in about 25% to about 80% by volume of the resinous binder composition). When the photogenerating component contains photoconductive compositions and/or pigments in the resinous binder material, the thickness of the layer typically ranges from about 0.1 to about 5.0 µm, or from about 0.2 to about 3 µm. The photogenerating layer thickness is often related to binder content, for example, higher binder content compositions typically require thicker layers for photogeneration. Thicknesses outside these ranges may also be selected.

In embodiments, the charge-generating layer includes a photoconductive pigment and a pigment sensitizing dopant having an electron acceptor molecule.

In embodiments, the photoconductive pigment is selected from the group consisting of vanadyl phthalocyanine, metal phthalocyanines, metal-free phthalocyanine, hydroxygallium phthalocyanine, titanyl phthalocyanine, chlorogallium phthalocyanine, benzimidazole perylene, amorphous selenium, trigonal selenium, selenium alloys, and mixtures and combinations thereof.

The dopant may comprise any suitable material having a suitable electron acceptor molecule. For example, the dopant is selected from the group consisting of 2,3-dichloro-5,6-dicyano-1,4-benzoquinone, tetracyanoethylene, 2,3,4,5-tetrabromobenzoquinone, 7,7,8,8-tetracyanoquinodimethane, chloranil, bromanil, 9-fluorenylidene, dinitroanthraquinone, p-nitrobenzonitrile, and mixtures and combinations thereof.

In embodiments, an imaging member is provided wherein the photoconductive pigment is chlorogallium phthalocyanine and the dopant is 2,3-dichloro-5,6-dicyano-1,4-benzoquinone; wherein the photoconductive pigment is hydroxygallium phthalocyanine and the dopant is 2,3-dichloro-5,6-dicyano-1,4-benzoquinone; wherein the photoconductive pigment is Type IV titanyl phthalocyanine and the dopant is 2,3-dichloro-5,6-dicyano-1,4-benzoquinone; wherein the photoconductive pigment is Type V titanyl phthalocyanine and the dopant is 2,3-dichloro-5,6-dicyano-1,4-benzoquinone, wherein the photoconductive pigment is Type B chlorogallium phthalocyanine and the dopant is tetracyanoethylene, wherein the photoconductive pigment is hydroxygallium phthalocyanine and the dopant is tetracyanoethylene, wherein the photoconductive pigment is Type IV titanyl phthalocyanine and the dopant is tetracyanoethylene, or wherein the photoconductive pigment is Type IV titanyl phthalocyanine and the dopant is tetracyanoethylene.

The dopant material may be provided in any suitable amount. In embodiments, the dopant is present in an amount selected from about 0.1 to about 40 weight % or from about 1 weight % to about 20 weight % based upon the total weight of charge generation layer.

In embodiments, the dopant is incorporated in the charge generation layer by (1) adding it into an already prepared charge generation layer dispersion; or (2) milling it together with polymeric binder and photoconductive pigment in solvents. In embodiments, the charge generation layer is coated from a charge generation dispersion that is prepared by adding the pigment sensitizing dopant having an electron acceptor molecule into the dispersion of a photoconductive pigment and a polymeric resin, or by ball milling the pigment sensitizing dopant having an electron acceptor molecule, a photoconductive pigment, and a polymeric resin together.

In embodiments, the dopant is substantially completely soluble in a charge generation layer solvent, comprising, for example, ketones, alcohols, aromatic hydrocarbons, halogenated aliphatic hydrocarbons, ethers, amines, amides, esters, and the like. Specific examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, among others.

As with the various other layers described herein, the photogenerating layer can be applied to underlying layers by any desired or suitable method. Drying, as with the other layers herein, can be effected by any suitable technique, such as, but not limited to, oven drying, infrared radiation drying, air drying, and the like.

The thickness of the imaging device typically ranges from about 2 to about 100 µm; from about 5 to about 50 µm, or from about 10 to about 30 µm. The thickness of each layer will depend on how many components are contained in that layer, how much of each component is desired in the layer, and other factors familiar to those in the art. In general, the ratio of the thickness of the charge transport layer to the charge generation layer can be maintained from about 2:1 to 200:1 and in some instances as great as 400:1. The charge transport layer, is substantially non-absorbing to visible light or radiation in the region of intended use but is electrically "active" in that it allows the injection of photogenerated holes from the photoconductive layer, i.e., charge generation layer, and allows these holes to be transported through itself to selectively discharge a surface charge on the surface of the active layer.

In embodiments, the at least one charge transport layer comprises from about 1 to about 7 layers. In embodiments, the at last one charge transport layer comprises a top charge transport layer and a bottom charge transport layer, wherein the bottom layer is situated between the charge generation layer and the top layer.

Aryl amines selected for the charge, especially hole transport layers, which generally are of a thickness of from about 5 to about 75 µm, or from about 10 to about 40 µm, include molecules of the following formula wherein X is alkyl, alkoxy, aryl, a halogen, or mixtures thereof, and especially those substituents selected from the group consisting of Cl and CH₃; and molecules of the following formula wherein X and Y are independently alkyl, alkoxy, aryl, a halogen, or mixtures thereof, alkyl and alkoxy contain for example from 1 to about 25 or from 1 to about 10 carbon atoms, such as methyl, ethyl, propyl, butyl, pentyl, and the corresponding alkoxides, aryl can contain from 6 to about 36 carbon atoms, such as phenyl, and the like, halogen includes chloride, bromide, iodide and fluoride. Substituted alkyls, alkoxys, and aryls can also be selected.

Examples of specific aryl amines include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine, and optionally mixtures thereof, and the like. Other known charge transport layer molecules can be selected. In embodiments, the charge transport layer comprises aryl amine mixtures.

In embodiments, the charge transport layer contains an antioxidant optionally comprised of, for example, a hindered phenol or a hindered amine.

Optionally, an overcoat layer can be employed to improve resistance of the photoreceptor to abrasion. An optional anticurl back coating may be applied to the surface of the substrate opposite to that bearing the photoconductive layer to provide flatness and/or abrasion resistance where a web configuration photoreceptor is desired. These overcoating and anticurl back coating layers are well known in the art, and can comprise for example thermoplastic organic polymers or inorganic polymers that are electrically insulating or slightly semiconductive. In embodiments, overcoatings are continuous and have a thickness of less than about 10 µm, although the thickness can be outside this range. The thickness of anticurl backing layers is selected to balance substantially the total forces of the layer or layers on the opposite side of the substrate layer.

Embodiments include a method of imaging which includes generating an electrostatic latent image on an imaging member, developing a latent image, and transferring the developed electrostatic image to a suitable substrate; methods of imaging and printing with the photoresponsive devices, including forming an electrostatic latent image on an imaging member; developing the image with a toner composition including, for example, at least one thermoplastic resin, at least one colorant, such as pigment, at least one charge additive, and at least one surface additive; transferring the image to a necessary member, such as, for example any suitable substrate, such as, paper; and permanently affixing the image thereto. In embodiments used in a printing mode, imaging methods include forming an electrostatic latent image on an imaging member by use of a laser device or image bar; developing the image with a toner composition including, for example, at least one thermoplastic resin, at least one colorant, such as pigment, at least one charge additive, and at least one surface additive; transferring the image to a necessary member, such as, for example any suitable substrate, for example, paper; and permanently affixing the image thereto.

An image forming apparatus for forming images on a recording medium comprises a) a photoreceptor member having a charge retentive surface to receive an electrostatic latent image thereon, wherein said photoreceptor member comprises a metal or metallized substrate, a charge generating layer comprising photoconductive pigment and a pigment sensitizing dopant having an electron acceptor molecule, and a charge transport layer comprising charge transport materials dispersed therein; b) a development component to apply a developer material to said charge-retentive surface to develop said electrostatic latent image to form a developed image on said charge-retentive surface; c) a transfer component for transferring said developed image from said charge-retentive surface to another member or a copy substrate; and d) a fusing member to fuse said developed image to said copy substrate.

Imaging members are provided wherein the charge generation layer is more sensitive than an imaging member having a comparable charge generation layer that is free of the dopant. For example, an imaging member herein provides a charge generation layer that is about 5 to about 15 % more sensitive than charge generation layer of a comparable device not comprising the present sensitized charge generation layer.

In embodiments, an imaging member having a charge generation layer comprising a dopant exhibits low imaging ghosting than an imaging member having a comparable charge generation layer that is free of the dopant.

### EXAMPLES

The following Examples are being submitted to further define various species of the present disclosure. These Examples are intended to be illustrative only and are not intended to limit the scope of the present disclosure. Also, parts and percentages are by weight unless otherwise indicated.

Example 1 and Comparative Example 1 were prepared as follows. Two multilayered photoreceptors of the rigid drum design were fabricated by conventional coating technology with an aluminum drum of 34 millimeters in diameter as the substrate. The two drum photoreceptors contained the same undercoat layer and charge transport layer. Comparative Example 1 contained a charge generation layer (CGL) comprising a film forming polymer binder and a photoconductive component, chlorogallium phthalocyanine; Example 1 contained the same layers as Comparative Example 1 except that 2,3-dicloro-5,6-dicyano-1,4-benzoquinone was incorporated into the charge generation layer.

The undercoat layer is a three-component undercoat which coating solution was prepared as follows: zirconium acetylacetonate tributoxide (35.5 parts), γ-aminopropyltriethoxysilane (4.8 parts) and poly(vinyl butyral) BM-S (2.5 parts) were dissolved in n-butanol (52.2 parts). The coating solution was coated via a ring coater, and the layer was pre-heated at 59°C for 13 minutes, humidified at 58°C (dew point = 54°C) for 17 minutes, and dried at 135°C for 8 minutes. The thickness of the undercoat layer was approximately 1.3 µm.
**Preparation of CGL dispersion for Comparative Example 1:** 2.7 gs of Type B chlorogallium phthalocyanine (CIGaPc) pigment was mixed with about 2.3 gs of polymeric binder VMCH (Dow Chemical), 30 gs of xylene and 15 gs of n-butyl acetate. The mixture was milled in an ATTRITOR mill with about 200 gs of 1 mm Hi-Bea borosilicate glass beads for about 3 hours. The dispersion was filtered through a 20-µm nylon cloth filter, and the solid content of the dispersion was diluted to about 5.8 weight percent with a mixture of xylene/n-butyl acetate=2/1 (weight/weight). The CIGaPc charge generation layer dispersion was applied on top of the above undercoat layer. The thickness of the charge generation layer was approximately 0.2 µm.
**Preparation of CGL dispersion for Example 1:** To the above CGL dispersion (Comparative Example 1) was added 0.25 gs of 2,3-dicloro-5,6-dicyano-1,4-benzoquinone, and the resulting dispersion was allowed to mix for at least 2 hours. The CIGaPc charge generation layer dispersion was applied on top of the above undercoat layer. The thickness of the charge generation layer was approximately 0.2 µm.

Subsequently, a 30-µm charge transport layer was coated on top of the charge generation layer, respectively, which coating dispersion was prepared as follows: N,N'-diphenyl-N,N-bis(3-methylphenyl)-1,1'-biphenyl-4,4'-diamine (5.38 g), a film forming polymer binder PCZ 400 [poly(4,4'-dihydroxy-diphenyl-1-1-cyclohexane, M_{w} = 40,000)] available from Mitsubishi Gas Chemical Company, Ltd. (7.13 g), and PTFE POLYFLON L-2 microparticle (1 g) available from Daikin Industries were dissolved/dispersed in a solvent mixture of 20 g of tetrahydrofuran (THF) and 6.7 g of toluene via CAVIPRO 300 nanomizer (Five Star technology, Cleveland, OH). The charge transport layer was dried at about 120°C for about 40 minutes.

The above prepared photoreceptor devices were tested in a scanner set to obtain photo-induced discharge cycles, sequenced at one charge-erase cycle followed by one charge-expose-erase cycle, wherein the light intensity was incrementally increased with cycling to produce a series of photo-induced discharge characteristic curves from which the photosensitivity and surface potentials at various exposure intensities were measured. Additional electrical characteristics were obtained by a series of charge-erase cycles with incrementing surface potential to generate several voltages versus charge density curves. The scanner was equipped with a scorotron set to a constant voltage charging at various surface potentials. The devices were tested at surface potentials of 700 V with the exposure light intensity incrementally increased by means of regulating a series of neutral density filters; the exposure light source was a 780 nm light emitting diode. The aluminum drum was rotated at a speed of 55 revolutions per minute to produce a surface speed of 277 mm per second or a cycle time of 1.09 seconds. The xerographic simulation was completed in an environmentally controlled light tight chamber at ambient conditions (40% relative humidity and 22°C). Two photo-induced discharge characteristic (PIDC) curves were generated. The PIDC results are summarized in Table 1. Incorporation of 2,3-dicloro-5,6-dicyano-1,4-benzoquinone into charge generation layer increased CIGaPc photosensitivity (initial slope of the PIDC) by about 15%, and decreased V (2.8 ergs/cm²), which represents the surface potential of the device when exposure is 2.8 ergs/cm², about 100 V.

The two devices were acclimated for 24 hours before testing in J zone (70°F and 10% humidity) for ghosting test. Print test was done in Copeland Work centre Pro 3545 using K station at t=500 print counts. Run-up from t=0 to t=500 print counts for the device was done in one of the CYM color stations. Ghosting levels were measured against TSIDU SIR scale (from Grade 1 to Grade 6). The smaller the ghosting grade (absolute value), the better the print quality. The ghosting results are also summarized in Table 1, and negative ghosting grades indicate negative ghosting. Incorporation of 2,3-dichloro-5,6-dicyano-1,4-benzoquinone into charge generation layer reduced ghosting by more than one grade.

**Table 1**

| | Sensitivity (Vcm²/erg) | V(2.8ergs/cm²) (V) | J zone ghosting (t=500) |
|---|---|---|---|
| Comparative Example 1 | -202 | 271 | -5 |
| Example 1 | -234 | 166 | -3.5 |

Example 2, 3 and Comparative Example 2 were prepared as follows. Three multilayered photoreceptors of the rigid drum design were fabricated by conventional coating technology with an aluminum drum of 34 mm in diameter as the substrate. The three drum photoreceptors contained the same undercoat layer and charge transport layer, and are same as described in the above two examples, however, charge generation layers are different. Comparative Example 2 contained a CGL comprising a film forming polymer binder and a photoconductive component, hydroxygallium phthalocyanine; Example 2 contained the same layers as Comparative Example 2 except that 2,3-dicloro-5,6-dicyano-1,4-benzoquinone was incorporated into the charge generation layer; Example 3 contained the same layers as Comparative Example 2 except that tetracyanoethylene was incorporated into the charge generation layer.
**Preparation of CGL dispersion for Comparative Example 2:** Three g of Type V hydroxygallium phthalocyanine (HOGaPc) pigment was mixed with about 2.0 g of polymeric binder VMCH (Dow Chemical), 45 g of n-butyl acetate. The mixture was milled in an ATTRITOR mill with about 200 g of 1 mm Hi-Bea borosilicate glass beads for about 3 hours. The dispersion was filtered through a 20 µm nylon cloth filter, and the solid content of the dispersion was diluted to about 5.8 weight % with n-butyl acetate. The HOGaPc charge generation layer dispersion was applied on top of the above undercoat layer. The thickness of the charge generation layer was approximately 0.2 µm.
**Preparation of CGL dispersion for Example 2:** To the above CGL dispersion (Comparative Example 2) was added 0.40 g of 2,3-dicloro-5,6-dicyano-1,4-benzoquinone, and the resulting dispersion was allowed to mix for at least 2 hours. The HOGaPc charge generation layer dispersion was applied on top of the above undercoat layer. The thickness of the charge generation layer was approximately 0.2 µm.
**Preparation of CGL dispersion for Example 3:** To the above CGL dispersion (Comparative Example 2) was added 0.25 g of tetracyanoethylen e, and the resulting dispersion was allowed to mix for at least 2 hours. The HOGaPc charge generation layer dispersion was applied on top of the above undercoat layer. The thickness of the charge generation layer was approximately 0.2 µm.

The three photoreceptors were tested for PIDC using the same procedure described as above. Three photo-induced discharge characteristic (PIDC) curves were generated. The PIDC results are summarized in Table 2. Incorporation of 2,3-dicloro-5,6-dicyano-1,4-benzoquinone into charge generation layer increased HOGaPc photosensitivity (initial slope of the PIDC) by about 5%, and decreased V (2.0 ergs/cm²), which represents the surface potential of the device when exposure is 2.0 ergs/cm², about 40 V. Incorporation of tetracyanoethylene into charge generation layer increased HOGaPc photosensitivity (initial slope of the PIDC) by about 10%, and decreased V (2.0 ergs/cm²), which represents the surface potential of the device when exposure is 2.0 ergs/cm², about 60 V.

**Table 2**

| | Sensitivity (Vcm²/erg) | V(2.0ergs/cm²) (V) |
|---|---|---|
| Comparative Example 2 | -390 | 140 |
| Example 2 | -405 | 98 |
| Example 3 | -420 | 80 |

Example 4, 5, 6 and Comparative Example 3 are prepared as follows. In Comparative Example 3, an imaging member was prepared by providing a 0.02 µm thick titanium layer coated on a biaxially oriented polyethylene naphthalate substrate (KALEDEX.TM. 2000) having a thickness of 89 µm (3.5 mils), and applying thereon, with a gravure applicator, a solution containing 50 g of 3-amino-propyltriethoxysilane, 41.2 g of water, 15 g of acetic acid, 684.8 g of denatured alcohol and 200 g of heptane. This layer was then dried for about 5 minutes at 135°C in the forced air drier of the coater. The resulting blocking layer had a dry thickness of 50 nm. An adhesive layer was then prepared by applying a wet coating over the blocking layer, using a gravure applicator, and which adhesive contains 0.2 % by weight based on the total weight of the solution of copolyester adhesive (Ardel D100 available from Toyota Hsutsu Inc.) in a 60:30:10 volume ratio mixture of tetrahydrofuran/monochlorobenzene/methylene chloride. The adhesive layer was then dried for about 5 minutes at 135°C in the forced air dryer of the coater. The resulting adhesive layer had a dry thickness of 20 nm.

A CGL dispersion was prepared by milling 1.65 g of the known polycarbonate lupilon 200 (PCZ-200) or Polycarbonate Z, weight average molecular weight of 20,000 available from Mitsubishi Gas Chemical Corp., 1.65 g of Type V titanyl phthalocyanine, 56.7 g of monochlorobenzene (MCB), and 150 g of GlenMills glass beads (1.0-1.25 mm in diameter) together via Attritor for 1.5 hours. The resulting dispersion was, thereafter, applied to the above adhesive interface with a Bird applicator to form a charge generation layer having a wet thickness of 6.4 µm (0.25 mil). A strip about 10 mm wide along one edge of the substrate web bearing the blocking layer and the adhesive layer was deliberately left uncoated by any of the charge generation layer material to facilitate adequate electrical contact by the ground strip layer that was applied later. The charge generation layer was dried at 120°C for 1 minute in a forced air oven to form a dry charge generation layer having a thickness of 0.4 µm.

This imaging member web was then overcoated with a two-layer charge transport layer. Specifically the charge generation layer was overcoated with a charge transport layer (the bottom layer) in contact with the charge generation layer. The bottom layer of the charge transport layer was prepared by introducing into an amber glass bottle in a weight ratio of 0.4:0.6 N,N'-bis(4-butylphenyl)-N,N'-di-p-tolyl-[p-terphenyl]-4,4"-diamine and Makrolon 5705^{RTM}, a known polycarbonate resin having a molecular weight average of from about 50,000 to 100,000 commercially available from Farbenfabriken Bayer A.G. The resulting mixture was then dissolved in methylene chloride to form a solution containing 15 % by weight solids. This solution was applied on the charge generation layer to form a coating of the bottom layer that upon drying (120°C for 1 minute) had a thickness of 14.5 µm. During this coating process the humidity was equal to or less than 15 %.

The bottom layer of the charge transport layer was overcoated with a top layer. The charge transport layer solution of the top layer was prepared as described above for the bottom layer. This solution was applied on the bottom layer of the charge transport layer to form a coating that upon drying (120°C for 1 minute) has a thickness of 14.5 µm. During this coating process the humidity was equal to or less than 15 %.

Example 4 is prepared by repeating the process of Comparative Example 3 except that to the charge generation layer dispersion of Comparative Example 3 is added 0.33 g of 2,3-dicloro-5,6-dicyano-1,4-benzoquinone.

Example 5 is prepared by repeating the process of Comparative Example 3 except that to the charge generation layer dispersion of Comparative Example 3 is added 0.33 g of tetracyanoethylene.

Example 5 is prepared by repeating the process of Comparative Example 3 except that to the charge generation layer dispersion of Comparative Example 3 is added 0.33 g of 9-fluorenylidene.

The four photoreceptors are tested for PIDC using the same procedure described as above. Incorporation of 2,3-dicloro-5,6-dicyano-1,4-benzoquinone, tetracyanoethylene or 9-fluorenylidene into charge generation layer increases TiOPc photosensitivity (initial slope of the PIDC) by from about 5% to about 20%.

## Claims

1. An imaging member comprising:
a substrate;
an optional undercoat layer;
a charge generation layer comprising photoconductive pigment and a pigment sensitizing dopant having an electron acceptor molecule; and
at least one charge transport layer.

2. The imaging member of claim 1, wherein the photoconductive pigment is selected from the group consisting of vanadyl phthalocyanine, metal phthalocyanines, metal-free phthalocyanine, hydroxygallium phthalocyanine, titanyl phthalocyanine, chlorogallium phthalocyanine, and mixtures and combinations thereof.

3. The imaging member of claim 2, wherein the photoconductive pigment is Type A chlorogallium phthalocyanine, Type B chlorogallium phthalocyanine, Type C chlorogallium phthalocyanine, Type V hydroxygallium phthalocyanine, Type IV titanyl phthalocyanine, or Type V titanyl phthalocyanine.

4. The imaging member of claim 1, wherein the pigment sensitizing dopant is selected from a group consisting of 2,3-dichloro-5,6-dicyano-1,4-benzoquinone, tetracyanoethylene, 2,3,4,5-tetrabromobenzoquinone, 7,7,8,8-tetracyanoquinodimethane, chloranil, bromanil, 9-fluorenylidene, dinitroanthraquinone, p-nitrobenzonitrile, and mixtures and combinations thereof.

5. The imaging member of claim 1 wherein the charge transport layer is comprised of aryl amine molecules, and which aryl amines are either of the formula wherein X is selected from the group consisting of alkyl, alkoxy, aryl and halogen, and said alkyl contains from 1 to 10 carbon atoms; or of the formula wherein each X and Y is independently selected from the group consisting of alkyl, alkoxy, aryl and halogen, wherein each alkoxy and each alkyl independently contains from 1 to 10 carbon atoms; aryl contains from 6 to 36 carbon atoms; and halogen is chloride, bromide, fluoride, or iodide.

6. The imaging member of claim 1, where in the at least one charge transport layer contains an antioxidant, preferably comprised of a hindered phenol or a hindered amine.

7. The imaging member of claim 1, wherein the at least one charge transport layer is comprised of a top charge transport layer and a bottom charge transport layer and wherein the bottom layer is situated between the charge generation layer and the top layer.

8. The imaging member of claim 1, wherein the charge generation layer is comprised of a photoconductive pigment, a polymeric resin and a pigment sensitizing dopant having an electron acceptor molecule.

9. A process for fabricating an imaging member comprising:
providing a substrate;
forming an optional undercoat layer on the substrate;
forming a sensitized charge generation layer comprising photoconductive pigment and a pigment sensitizing dopant having an electron acceptor molecule; and
forming at least one charge transport layer.

10. An image forming apparatus for forming images on a recording medium comprising:
a) a photoreceptor member having a charge retentive surface to receive an electrostatic latent image thereon, wherein said photoreceptor member comprises a metal or metallized substrate, a charge generation layer, and at least one charge transport layer; wherein the charge generation layer comprises a photoconductive pigment and a pigment sensitizing dopant having an electron acceptor molecule;
b) a development component to apply a developer material to said charge-retentive surface to develop said electrostatic latent image to form a developed image on said charge-retentive surface;
c) a transfer component for transferring said developed image from said charge-retentive surface to another member or a copy substrate; and
d) a fusing member to fuse said developed image to said copy substrate.
